

## UNITED STATES PATENT OFFICE

1,951,712

## PROCESS FOR IMPROVING FIBROUS MATERIALS

Conrad Schoeller, Ludwigshafen-on-the-Rhine, Germany, assignor to I. G. Farbenindustrie Aktiengesellschaft, Frankfort - on - the - Main, Germany

No Drawing. Application May 21, 1930, Serial No. 454,515. In Germany May 30, 1929

13 Claims. (Cl. 8—20)

The present invention relates to a process for improving fibrous materials.

Many fibrous materials, especially artificial fibres have a small flexibility and softness which reduce their range of application, and even with materials which are already flexible and soft an increase in these properties is frequently desirable.

I have now found that an excellent softness and flexibility may be imparted to fibrous materials of all kinds, in particular artificial fibres and especially the different kinds of artificial silk, by treating them with aqueous solutions of sulphonated aliphatic carboxylic acids of high molecular weight which term is meant to include the water-soluble salts of the same, or by incorporating them with the said sulphonated acids. The fibres treated in this manner are extremely soft and agreeable to the touch.

20 Suitable sulphonated acids are those of the following general structure



wherein R is the hydrocarbon radical of a saturated aliphatic carboxylic acid of high molecular weight such as palmitic, stearic, lauric or myristic acids, or similar saturated acids as occur in fats 30 or oils of vegetable or animal origin and in oxidation products of solid or liquid paraffin wax. The quantities of the sulphonated acids or their salts employed are usually from 1 per thousand to say 5 per cent of the aqueous solutions with which 35 the fibres are treated and in most cases solutions of 0.2 to 1 per cent fulfill all requirements. Artificial fibres to be softened may be prepared by any process such as by the different processes of producing viscose silk, by the Chardonnet or 40 Pauly processes or by air spinning processes of nitrocellulose or cellulose carboxylates. In any case very good results are obtained and the fibres treated do not contain foreign matter, such as the oils hitherto employed for softening purposes, which must be removed subsequently from 45 the fibres in most cases when the fibres are to be worked further. The process according to the present invention may be combined with other processes of improving fibrous materials in which 50 the fibres are usually hardened or stiffened to some degree as for example in sizing and in many cases of dyeing; in these cases it is sufficient to add the quantities mentioned above of the sulphonated acids or their salts to the sizing or dyeing liquors. The treatment of the fibres is pref-

erably carried out while warming to temperatures which, preferably, do not exceed the boiling point of the solutions.

The following examples will further illustrate the nature of this invention, but the invention is not restricted thereto.

## Example 1

Cuprammonium silk is treated in a solution which contains 0.5 gram of the monosodium salt 65 of palmitic sulphonated acid or of stearic sulphonated acid per litre for 20 minutes at from 50° to 60° centigrade, centrifuged and dried. The silk treated in this manner is extremely soft and agreeable to the touch. Similar results can be 70 obtained with sulphonated acids, or their salts, of lauric or myristic acids or mixtures of the sulphonated acids.

## Example 2

A dyeing vat for artificial silk from viscose is 75 prepared from a 2 per cent aqueous solution of brilliant benzo green B 1.5 gram of the monosodium salt of the sulphonated acid of palmitic acid being added to each litre of the bath. After dyeing in the manner usually applied when dyeing with substantive dyestuffs, the silk is rinsed, 80 centrifuged and dried. The artificial silk has a very soft and supple touch.

## Example 3

A mixed fabric of cotton and artificial silk from cellulose acetate is treated for 20 minutes at from 50° to 55° C. with a solution of 5 grams of the salt of triethanol amine with the sulphonated acid of stearic acid in 1 litre of water whereupon 90 the fabric is centrifuged and dried. The fabric is rendered much more supple than it was originally.

## Example 4

Hanks of artificial silk are treated for a quarter of an hour at from 40° to 50° C. with a solution of 10 grams of glue or of soluble starch and 3 grams of the salt of triethanol amine with the sulphonated acid of palmitic or stearic acid whereupon 100 the hanks are centrifuged and dried. The artificial silk which becomes hard and brittle by a treatment with glue or starch solution is rendered elastic and supple by the addition of the sulphonated acid salt and possesses a high smoothness 105 particularly advantageous on weaving the silk.

## Example 5

Yarn for making stockings from mercerized cotton or a yarn spun from short fibres of arti- 110

ficial silk and known in the trade under the name "Vistra" is treated at about 40° C. for a quarter of an hour with an aqueous 0.1 per cent solution of the di-sodium salt of the sulphonic acid of palmitic acid, whereupon the yarn is centrifuged and dried. The smooth yarn obtained can be easily wound on bobbins and passes very smoothly through the weaving needles, the passage of the yarn through a particular oiling device, which is necessary without the aforesaid treatment, being superfluous. The woven stockings possess a particularly soft touch.

What I claim is:—

1. The process of rendering artificial silk soft and flexible which comprises treating the silk with an aqueous solution of a substance of the class consisting of compounds of the following general structure

20



wherein R is the hydrocarbon radical of a saturated aliphatic carboxylic acid of high molecular weight, and the water soluble salts of said compounds.

2. The process of rendering artificial silk soft and flexible which comprises treating the said material with an aqueous solution comprising from 0.1 to 5 per cent strength of a sulphonic acid of the following general structure

35



wherein R is the hydrocarbon radical of a saturated aliphatic carboxylic acid of high molecular weight.

40 3. The process of rendering artificial silk soft and flexible which comprises treating the said material with an aqueous solution of from 0.2 to 1 per cent of a sulphonic acid of the following general structure

45



wherein R is the hydrocarbon radical of a saturated aliphatic carboxylic acid of high molecular weight.

45 4. The process of rendering artificial silk soft and flexible which comprises treating the said materials with an aqueous solution of from 0.2 to 1 per cent of a sulphonic acid of the following general structure

60



wherein R is the hydrocarbon radical of a saturated aliphatic carboxylic acid of high molecular weight while warming.

65 5. The process of rendering artificial silk soft and flexible which comprises treating the said material with an aqueous solution comprising a sulphonic acid of the following general structure

70



wherein R is the hydrocarbon radical of a saturated aliphatic carboxylic acid of an animal fat,

6. The process of rendering artificial silk soft and flexible which comprises treating the said material with an aqueous solution, of from 0.2 to 1 per cent strength, of a sulphonic acid of the following general structure

80



wherein R is the hydrocarbon radical of palmitic acid.

7. The process of rendering artificial silk soft and flexible which comprises treating the said material with an aqueous solution, comprising from 0.2 to 1 per cent of a water-soluble salt of a sulphonic acid of the following general structure

90



wherein R is the hydrocarbon radical of palmitic acid.

8. As a new article, soft artificial silk, the single fibres of which have a thin superficial coating comprising a substance of the class consisting of compounds of the following general structure

100



wherein R is the hydrocarbon radical of a saturated aliphatic carboxylic acid of high molecular weight, and the water soluble salts of said compounds.

9. As a new article of manufacture, soft artificial silk, the single fibres of which have a thin superficial coating comprising a sulphonic acid of the following general structure

115



wherein R is the hydrocarbon radical of a saturated aliphatic carboxylic acid of high molecular weight.

10. As a new article of manufacture soft artificial silk, the single fibres of which have a thin superficial coating comprising a sulphonic acid of the following general structure

125



wherein R is the hydrocarbon radical of palmitic acid.

11. As a new article of manufacture, soft artificial silk, the single fibres of which have a thin superficial coating comprising a water soluble salt of a sulphonic acid of the following general structure

130



wherein R is the hydrocarbon radical of a saturated carboxylic acid of an animal fat.

12. As a new article of manufacture, soft artificial silk, the single fibres of which have a thin superficial coating comprising a water-soluble

140

150

salt of triethanol amine with a sulphonic acid of the following general structure



wherein R is the hydrocarbon radical of a carboxylic acid of an animal fat.

13. As a new article of manufacture, soft artificial silk, the single fibres of which have a thin

superficial coating comprising a water-soluble salt of triethanol amine with a sulphonic acid of the following general structure



wherein R is the hydrocarbon radical of palmitic acid.

CONRAD SCHOELLER. 85

15

90

20

95

25

100

30

105

35

110

40

115

45

120

50

125

55

130

60

135

65

140

70

145

75